

Sept. 2, 1930.

H. R. VAN DEVENTER

1,774,856

MAGNETIC DEVICE

Filed April 22, 1924

*Fig. 1.*



*Fig. 2.*



*Fig. 3.*



*Fig. 4.*



INVENTOR  
Harry R. VanDeventer  
BY  
ATTORNEY

*M. J. Presson*

## UNITED STATES PATENT OFFICE

HARRY B. VAN DEVENTER, OF NEW YORK, N. Y., ASSIGNOR TO DUBILIER CONDENSER CORPORATION, OF NEW YORK, N. Y., A CORPORATION OF DELAWARE

## MAGNETIC DEVICE

Application filed April 22, 1924. Serial No. 708,313.

This invention relates to improvements in magnetic devices; especially devices to afford electrical and magnetic conductance in signalling and other electrical arts.

5 An object of the invention is to provide a magnetic device of novel construction with constituent parts which have relatively great thinness and can easily be produced; the device being capable of affording sufficient magnetic conductivity and keeping the losses at a 10 minimum in actual operation.

Another object of my invention is to provide a laminated magnetic core which substantially reduces eddy current and hysteresis 15 losses, and is, therefore, particularly adapted for use in devices employed in high frequency circuits.

I desire my invention to be understood as including a magnetic device having the characteristics above mentioned; the parts or elements thereof, and the method by which such a device and the parts composing it are produced.

Other objects and advantages of my invention will appear from the following description and the peculiar features thereof are defined in the appended claims; but I of course reserve the right to vary the details of structure or proceeding herein specifically set forth, to the full extent compatible with the broad meanings of the terms in which the claims are expressed.

In the drawing Fig. 1 shows a magnetic core constructed in accordance with my invention;

35 Fig. 3 is an exploded view of Fig. 1; and Figs. 2 and 4 show other forms of magnetic cores.

In the practice of my invention, I take a thin sheet of some insulating substance, which may be fibrous material, such as paper, and spread thereon a sufficient quantity of finely divided particles to form a continuous layer. The particles must be iron or something else 45 that is both electrically and magnetically conductive, and are distributed evenly over the surface of the sheet and caused to adhere thereto. At the same time the iron particles must be attached to the paper close enough to 50 one another to be all in contact, thus giving

continuity to the layer and eliminating open spaces or air gaps. To spread the metallic particles over the surface of the paper, any feasible method can be chosen. For example, I may make use of the well known Schoop process, by which iron dust is blown or sprayed against the paper, being forcibly impelled against the surface thereof and caused to fill the microscopic recesses or depressions in same, and to stick to the fibers of the paper, 55 and thus afford a thin or tenuous layer covering the paper over its entire extent. The process may be performed in an atmosphere of nitrogen, carbon dioxide, or some other medium that will not support combustion, to 60 prevent oxidation of either the metallic particles or the paper.

The paper may be in the form of strips or sheets, and may thus be covered with a continuous thin layer of particles on one side or 70 both. After covering, the laminated element so produced can be coated with thin varnish or any other suitable non-conducting substance to protect its surface, keep the layer from being rubbed off, and to add some stiffness to the element when dried after coating. The strip or sheet with the layer thereon can be trimmed when finished and cut into laminated elements of the required length and 75 width.

To make a magnetic core for transformers or coils out of such elements, for instance, a number of elements are superposed one upon another and bound together. The elements may consist of a sheet of paper with a magnetic layer on one side with or without a non-conductive coating; because if the elements are assembled with the untreated surface of the paper of one against the metallic layer of another, the magnetic layers of the entire core 80 will be effectually isolated from one another; but when given magnetic layers on both sides of the paper, each element must have a non-conductive coating all over it.

Figs. 1 and 2 show well known forms of a 85 magnetic core for windings 3 in which the elements 1 and 2 are made in accordance with my invention and are built to form a laminated core. The element 1 may be coated on one side only and thus its coating separated 90

from 2, or if varnish is used to cover the magnetic material both sides may be coated, the varnish serving to laminate the core. The laminated effect is shown by the exploded view of Fig. 3.

With my invention laminated elements of relatively small thinness can be made, and yet have the necessary permeability while keeping the eddy current and other losses to the smallest possible amount.

Due to the very high frequency currents employed in radio circuits, very considerable eddy current and hysteresis losses are incurred when the usual type of core is used, and my construction is therefore particularly adapted for use in radio apparatus.

Instead of blowing or spraying the magnetic dust or particles against the paper, I may obtain such particles by precipitation from a liquid containing a solution of some compound in which the iron or the like occurs; and then spreading the precipitate out thinly over the insulating sheet in any manner capable of yielding the desired results; or the magnetic particles can be precipitated directly upon the sheet, deposited in a continuous layer distributed all over the surface.

Instead of making laminations for magnetic cores, I may also employ long and relatively narrow strips 4 of thin insulating material covered in the manner above set forth with a layer of iron particles, and then wind the strip into a roll or spiral, as shown diagrammatically in Fig. 4. This roll can be employed either as a magnetic core or as a coil for the passage of electric current, such as a loading inductance coil in radio, or in signalling with wires.

When paper is used to receive the layer of particles, a binder may be utilized to make the particles adhere to the paper. For this purpose, the paper may be covered or lightly impregnated with a thin soft wax, and when the particles come into contact with the wax they stick to it. After the layer is fully formed, the paper and the layer can be rolled, compressed, or squeezed, both to expel the surplus wax and to make the final product thinner.

Instead of paper, thin sheets or strips of any other suitable material may be utilized to receive the layer of particles. For example, I may take some of the compounds of cellulose, such as are employed in making films for photography, and treat the surface thereof with a liquid capable of dissolving the film, but only to the extent of making the surface sticky, so that the magnetic particles will adhere; or I may take the thin gelatinous substance which is attached to a photographic film to give it the light-sensitive coating, and cover this film with the magnetic layer under conditions which will permit adhesion to take place. In any case

the thin strip or sheet with the conductive layer may be varnished or not, as desired.

By this invention conductive elements in the form of laminations or strips to be rolled, can be produced having a thinness of a quarter or a half of a mil, or one-thousandth of an inch.

Having described my invention, what I believe to be new and desire to secure and protect by Letters Patent of the United States is:—

1. A magnetic core made up of laminated elements superposed one upon another, each element comprising a thin layer of magnetic material consisting of finely divided particles in contact with one another, giving continuity to the layer, and insulation between the layers, said particles being held by adhesion to one another and to said insulation. 80

2. A core for electro-magnetic apparatus comprising a plurality of elements in the form of thin plates which are insulated from one another, each element including a non-magnetic carrier sheet upon which there is deposited finely divided magnetic material. 85

3. A core element for electro-magnetic apparatus, consisting of a sheet of non-metallic material having a coating of finely divided particles of ferro-magnetic material. 90

4. A core element for a magnetic circuit in a high frequency apparatus consisting of a lamina of non-magnetic material, one or more of the surfaces of said lamina being coated with a highly divided deposit of magnetic material. 95

5. A core for electro-magnetic apparatus comprising a sheet of insulating material having a coating of finely divided particles of ferro-magnetic material. 100

6. A core for electro-magnetic apparatus comprising a sheet of flexible insulating material having a coating of finely divided particles of ferro-magnetic material. 105

In testimony whereof I affix my signature.

HARRY R. VAN DEVENTER. 110

115

120

125

130